

R. B. MANLEY.  
ABRASIVE PAPER AND CLOTH.  
APPLICATION FILED MAR. 31, 1915.

1,161,497.

Patented Nov. 23, 1915.



WITNESSES

R. A. Alderson  
José B. Heller.

INVENTOR

R. B. Manley,  
by Bahewell, Paymer, Parmer  
Atteys.

# UNITED STATES PATENT OFFICE.

RALPH B. MANLEY, OF NIAGARA FALLS, NEW YORK, ASSIGNOR TO THE CARBORUNDUM COMPANY, OF NIAGARA FALLS, NEW YORK, A CORPORATION OF PENNSYLVANIA.

## ABRASIVE PAPER AND CLOTH.

1,161,497.

Specification of Letters Patent. Patented Nov. 23, 1915.

Original application filed April 22, 1913. Serial No. 762,827. Divided and this application filed March 31, 1915. Serial No. 18,322.

To all whom it may concern:

Be it known that I, RALPH B. MANLEY, a citizen of the United States, residing at Niagara Falls, in the county of Niagara and State of New York, have invented a new and useful Improvement in Abrasive Paper and Cloth, of which the following is a full, clear, and exact description, reference being had to the accompanying drawings, forming part of this specification, in which the figure is a side elevation, partly diagrammatic, of one form of apparatus which may be employed in the manufacture of the paper and cloth.

My invention relates to abrasive paper and cloth and provides an article of this character having a greater degree of flexibility imparted thereto than has heretofore been possible.

Abrasive paper and cloth of the character to which my invention relates, consists of grains of abrasive material, such as carborundum, aloxite, flint, garnet, emery and other similar materials, which are fastened to a backing of paper or cloth by means of glue or other adhesives. This material is widely used in the grinding and polishing of metal, leather, wood and a variety of other substances. When abrasive paper or cloth of this character is made up with sufficient

glue to properly hold the abrasive grains, and is properly dried, it can be flexed or bent to a certain extent, depending upon the amount and character of the glue and of the abrasive grains and other conditions, but it cannot be bent at very short angles on account of the stiffness of the glue. If this is attempted, it results in the glue and adhesive grains peeling off in large flakes. For

many purposes, it is highly desirable that this paper shall possess a very considerable degree of flexibility. For instance, emery cloth is often used by machinists in various classes of hand work where it is necessary to reach curved and irregular surfaces of small section. In the wood-working industry, garnet paper is placed around the drums of sanding machines, and if the paper is stiff and lacks flexibility, it will not lie close to

the surface of the drum. This frequently results in an irregular cylindrical abrasive surface, and if the paper is forced into contact with the drum its structure is injured so that it begins to peel off quickly when

subjected to use. The finishing paper used by cabinet makers when smoothing wood should also possess a high degree of flexibility. It has been attempted to obtain this degree of flexibility in various ways, as by the use of various grades of glue and the addition of different substances to the glue. None of these methods have, however, been entirely successful. For instance, the addition of such substances to the glue prevents it from properly drying or remaining perfectly dry and also results in the loss of adhesive power.

My invention overcomes these difficulties and produces an abrasive paper or cloth which is capable of being bent or flexed to a large degree without injury thereto. I produce this result by mechanical treatment of the paper or cloth in such a manner that the adhesive bond is broken at substantially regular intervals along the surface of the backing in a direction normal to the backing and in a manner to impart this flexibility.

While my improved method may be carried out in various ways and by the use of apparatus of various kinds, I have in the accompanying drawings illustrated one form of apparatus which I have found to be highly satisfactory and which will now be described.

In this drawing, 2 designates the frame of the machine, which carries two endless belts 3 and 4, both of which are shown as driven by the respective drive belts 5 and 6 from any suitable source of power. These belts 3 and 4 are disposed in the following manner. The belt 4 is carried over the driven pulley 7, and thence over the flexing member 8. This flexing member may be a metal bar of rectangular or other section so as to present a suitable sharp corner over which the backing of the abrasive cloth or paper can be drawn and bent to the required degree. It may also consist of a round bar or roll of relatively small diameter. The belt 3 runs over the driving pulley 13, and the idler wheel 9, thence over the flexing member 8 on top of the belt 4 and thence over the idler 10 and back to the driving pulley 13. 11 designates the roll of paper or cloth to be treated. This is led with its grain side up between the belts 3 and 4 and over the flexing member 8 to the rewinding roll 12, which is also driven by

suitable means, such as the belt 14. Means of any suitable or well known character may be provided for adjusting the tension of both belts 3 and 4. The driving belt 6 can 5 be dispensed with, and it is also possible to dispense with the belt 4 and to permit the paper to slide directly over the flexing member with its grain side out without the assistance of the under belt.

10 The effect of passing the paper or cloth over the flexing member is to break the adhesive bond (which may be of any approved character) at substantially regular intervals along the surface of the backing in a direction normal to the backing and in such a manner that the flexibility is very greatly increased.

I have found from actual practice that when garnet paper, for instance, is treated 20 in this manner, it can be run on a drum sander from three to four times as long as ordinary paper without peeling.

The degree of flexibility which is obtained 25 is proportional to the frequency of the breaks; that is, the more breaks per lineal inch, the greater is the flexibility. Care, however, should be taken that the breaks are not too close together, as this overcomes the adhesion of the grain and makes the cloth 30 or paper useless for many purposes. The number of breaks, per lineal inch, will vary with cloth and paper of different grits, but I

have found that the breaks, in order to give proper flexibility, should in all cases be not less than five and not more than twenty per 35 lineal inch.

My invention has also proved to be of great assistance in increasing the efficiency and prolonging the life of emery cloth and aloxite cloth, which are used in certain operations of finishing machinery. It has also proved very useful in treating garnet cloth to be used for garnet belts in the finishing of molded surfaces. It prevents the peeling 40 of paper for use in heel-scouring in the 45 shoe industries. It has, of course, many other useful applications.

This application is a division of my co-pending application Serial No. 762,827, filed April 22, 1913.

50

I claim:

As a new article of manufacture, an abrasive-coated backing, in which the abrasive bond of the coating material has been mechanically broken or flexed so as to give not less than five nor more than twenty breaks per lineal inch, substantially as described.

55 In testimony whereof, I have hereunto set my hand.

RALPH B. MANLEY.

Witnesses:

FRANK H. MANLEY,  
GEORGE N. ALLEN.